

Patented Aug. 4, 1925.

1,548,514

# UNITED STATES PATENT OFFICE.

GASTON DE DUDZEELE, OF PARIS, FRANCE.

## TREATMENT OF METALS TO BE DRAWN, WIREDRAWN, OR ROLLED.

No Drawing.

Application filed February 26, 1923. Serial No. 621,472.

To all whom it may concern:

Be it known that I, GASTON DE DUDZEELE, a subject of the King of Belgium, residing at 12 Avenue Bugeaud, Paris, France, have invented certain new and useful Improvements in the Treatment of Metals to be Drawn, Wiredrawn, or Rolled, of which the following is a specification.

For the purpose of drawing, wire-drawing or rolling metals in order to bring them to the required shape and dimensions, the metal requires to be annealed, cleaned and eventually coppered between each operation or "pass." It has however been recognized that all these intermediary operations may be suppressed by previously coating the metals with a thin layer of lead, but it is advisable, in order to obtain good results, for the lead to be as pure as possible so as to retain all its properties of malleability and it is necessary that the lead should impregnate effectively the metal to be worked, so that during the working of it, the layer of lead will not separate from it.

By electrolytic or chemical means it is possible to obtain a coating of perfectly pure lead, but the adhesive qualities of this coating are not satisfactory, as this pulverulent and crystalline deposit is easily removed; moreover the electrolytic or chemical process is not economical as it requires an expensive plant and careful and constant supervision.

Hot dipping, as actually practiced, therefore appears, at first sight, well adapted to replace electrolytic or chemical coating, but up to the present a layer of pure lead could not be deposited by the ordinary method on iron and copper, for example, these metals having no chemical affinity for lead. It has been proposed, for ensuring a slow but sufficient deposit of lead, to incorporate in the latter metal a sufficiently effective quantity (5 to 10%) of tin or antimony. However tin and antimony harden lead to such an extent that the ordinary coating process cannot be applied to the mechanical working of metals.

The chief feature of the present invention consists in the possibility of rolling, drawing or wire-drawing metals without any intermediary operations by causing on such metals an effective impregnation of lead by means of first amalgamating the metal to be worked and then lead coating it by immersion in molten lead or any of its alloys.

The mercury presents the following advantage: the instantaneous impregnation of the lead. It may be mentioned that a metal treated as described is not simply covered with a more or less thin sheath of lead liable to be removed or worn off during the drawing or rolling operations, but the lead impregnates the metal itself, thus preventing the drawing or rolling from causing a direct friction of the die, ring, or roller on the metal to be worked. Up to the end of the rolling or drawing operations, the lead exerts its regulating influence.

The function of the mercury salt is not only to increase the chemical affinity between the metal to be treated and the lead, but further to give to the metal thus treated such qualities as make it possible to draw or roll it several times without altering its qualities of resistance, elongation, etc., this not being the case when working a non-amalgamated metal.

The amalgamation may be effected by immersing the metals to be drawn, rolled or otherwise worked in a solution of a suitable mercury salt.

Amongst others a bath composed as follows gives excellent results:

1 gallon of a dilute solution of hydrochloric acid at 6° Baumé, saturated with ammonium chloride, and 1½ ounce of mercury chloride.

After remaining a few seconds in this bath, the metallic articles have acquired a grey colour due to the formation of a complex amalgam. They are then withdrawn from this bath and dipped directly into pure molten lead.

The lead coated articles are allowed to cool and may then be drawn, rolled or wire-drawn without the necessity of any intermediary operation such as annealing, cleaning or coppering afresh between each operation or pass.

It is to be understood that by the expression "mechanically working metals" in the appended claims, it is intended to cover drawing, wire-drawing and rolling metals.

What I claim is:

1. A process for mechanically working metals to change their form, comprising, amalgamating a metal starting piece to be worked into a different form, coating the piece with lead, and then mechanically working the lead-coated metal starting piece into its changed finished form.

2. A process for mechanically working metals to change their form, comprising, treating the surface of a metal starting piece to be worked into a different finished form  
5 with a solution of a mercury salt capable of amalgamating the surface, dipping the metal starting piece into pure molten lead, and then mechanically working the lead-coated metal piece into its different finished  
10 form.

3. A process for drawing metals, comprising, amalgamating the metal to be drawn, then coating it with lead, and then mechanically drawing the lead-coated metal.

In testimony whereof I have signed my <sup>15</sup> name to this specification.

GASTON DE DUDZEELE.

Witnesses:

T. ARMENGAUD,  
H. DEFÈVREMONT.